

July 20, 1943.

O. J. KRUEGER ET AL.

2,324,519

## DRYING OF DISTENDED FIBROUS PRODUCTS

Filed Aug. 3, 1940

2 Sheets-Sheet 1



Inventors:  
Otto J. Krueger and  
John Caresio  
By: Dyke and Schaines Atty's.

July 20, 1943.

O. J. KRUEGER ET AL

2,324,519

DRYING OF DISTENDED FIBROUS PRODUCTS

Filed Aug. 3, 1940

2 Sheets-Sheet 2



Inventors:  
Otto J. Krueger and  
John Caresio  
By: Dyke and Schaines  
*Atlys.*

## UNITED STATES PATENT OFFICE

2,324,519

## DRYING OF DISTENDED FIBROUS PRODUCTS

Otto J. Krueger, Western Springs, and John Caresio, Chicago, Ill., assignors to Masonite Corporation, a corporation of Delaware

Application August 3, 1940, Serial No. 351,030

4 Claims. (Cl. 34—7)

The invention relates to the drying of distended fibrous products, and relates more particularly to the drying of such products made from fibrous materials such as kraft pulp, having for example foaming agents such as saponin mixed therewith and the mixture agitated with provision for air supply, serving to produce a condition wherein relatively stable bubbles are incorporated with the fibers of the pulp in such manner as to produce distention and maintain the fibres in distended relation, in which relation they are fixed by drying.

The principal object of the invention is the provision of an improvement in the drying of distended fibrous products by means of heated air and products of combustion whereby an improved product can be made, and increased speed of production obtained.

When relatively thick sheets, as for example, sheets one inch thick of distended fibrous material and containing a considerable proportion of water are traveled along on a reticulated support, as a Fourdrinier screen, with excess or free water leaving the sheet from the bottom, the content of water retained in the sheet is least at and near the top surface, and the water content increases downwardly and is greatest at and near the bottom of the sheet.

No great difficulty is encountered in drying the lower part of such a sheet by passing it through a hot air drier and subjecting it therein to temperatures sufficiently high to secure rapid drying and good qualities in the sheet, without scorching or burning. The lower surface of the sheet is shielded to some extent by the wire belt on which it is taken through the drier, and also by the roller supports for supporting the belt. It is also more or less protected by water vapor formed from the water in this part of the sheet. The water in this part of the sheet appears to give good heat conductivity, so that the heat is effectively conducted within the interior of this part of the sheet, and the drying extends upwardly into the sheet from beneath.

If, however, the sheet is dried in a comparatively short drier, which can be operated at high temperature, the same speed of travel which gives good results at and near the bottom of the sheet because of considerations as above described will cause the upper surface of the sheet to be charred or even burned, and at and about the median zone of the sheet the drying will not be complete.

This is apparently due to the relatively low water content in the upper part of the sheet. The upper part of the sheet lacks the shielding

which the lower part of the sheet gets from the carrying belt; blanketing of this upper part of the sheet by water vapors is less than for the lower part of the sheet because there is less water present to be vaporized; and heat conducted from the upper surface of the sheet downwardly is decreased relative to the corresponding effect at and near the bottom of the sheet, because of decreased heat conductivity due to reduced water content.

Consequently in the hot air drying of light weight sheets of distended fibrous materials, it has been necessary to keep the temperatures no higher than can be withstood by the upper surface of the sheet without charring or burning, and this in turn has made it necessary to keep production speed correspondingly low or to make use of very long and highly expensive drying apparatus. These difficulties are avoided by the present invention through the addition of water to the top surface and upper part of the sheet prior to its introduction into the drier.

By the addition of such water the temperatures are no longer limited by the ready charring of the upper surface, as is the case without the added water. A small proportion of fire retarding material, such as boric acid for example, can advantageously be dissolved in and supplied to the top of the sheet with such added water, but good results can be obtained with or without such dissolved soluble material. It might be supposed that such addition of water or water containing boric acid or other fire retarding material would slow down the drying and increase the fuel cost of drying, but the reverse of this is really the case. In the drying of the sheet, water vapor is developed rapidly at the top surface of the sheet to which added water has been supplied, and this vapor appears to have a protecting effect against ready charring. The heat penetrates downwardly into the interior of the sheet or board, as is evidenced by thorough drying throughout the sheet. This effect appears to be produced by the greater heat conductivity due to the presence of the water added to the sheet from above. The fuel cost can be reduced, notwithstanding the fact that more water has to be dried out, and this again appears to be due to the added water by which heat is conducted into the interior of the board from above, such heat conduction effect and the drying of the inner part of the sheet being the more efficient since effective heat conduction to the interior of the sheet takes place not only from the bottom of the sheet upwardly, but also downwardly from the top of the sheet.

It is thus an object of the invention to secure uniform drying of the sheets of distended fibrous material through the indirect, but nevertheless effective route by adding to the quantity of water which has to be dried out of the sheet.

The accompanying drawings forming a part of the specification show an illustrative embodiment of apparatus for carrying out the invention. In said drawings,

Fig. 1 is a schematic side view of forming apparatus and also showing a portion of the drying apparatus;

Fig. 2 is a side view on an enlarged scale of spraying apparatus;

Fig. 3 is a cross-section on line 3—3 of Fig. 2;

Fig. 4 is a side view of a part of a drier; and

Fig. 5 is a cross-sectional view on line 5—5 of Fig. 4.

Referring first to Fig. 1, reference character 10 designates a flow box to which the mix, consisting preferably of fiber, foaming agent, sizing materials, water and air from which the sheet is to be formed, is supplied through the pipe 12. This mix is kept in agitation by an agitator 14, located behind the intermediate dam 16 in the flow box, and after passing over the dam 16 the mix is further agitated by the roll agitator 20. The mix from the flow box is delivered through the passage 18 on to the Fourdrinier wire 22, the depth of the layer so delivered being regulated by a slice plate 24, which can be adjusted for height and for thickness of sheet, as by the regulating screws 26. The upper run 27 of the Fourdrinier wire 22 is supported in the usual manner by means of the spaced rollers 28 shown only in part but provided throughout the length of the Fourdrinier wire belt, and the sheet formed from the mix is designated by reference character 30. At the respective ends of the forming apparatus the Fourdrinier wire 22 runs around a breast roll 32, and a couch roll 34. The return or under-run 36 of the Fourdrinier wire 22 runs over rollers 38 and beneath other rollers as 40, which may be made adjustable and used for tensioning the Fourdrinier wire as indicated by the arrows 40' placed near these rolls. Suction boxes 41, 41 may be provided, if desired, for compacting the extreme lower portion of the sheet 30 somewhat in order to give increased strength to this part of the sheet. The roll 34 is preferably perforated, and air under light pressure supplied at the interior thereof to ensure that the sheet 30 is freed from the Fourdrinier wire 22.

Transfer means are provided for delivering the formed sheet from the Fourdrinier wire to the drier belt, as it passes off the Fourdrinier wire belt and over the couch roll 34, and may consist, in the simplest form, of a short transfer belt 42, running over the rollers 44, 44, 44 arranged in triangular relation so as to guide the belt 42 to perform the transfer function.

The drying mechanism is illustrated only in part. This drying mechanism, which is of the hot air type and does the drying by circulating heated gases including products of combustion, is preferably composed of several sections, the number of sections and total length of the drier varying with the conditions for the particular installation, and in the showing herein made, the first and second sections only are illustrated. Such drier comprises essentially a long drying chamber or tunnel 50, and heating and air circulating chambers which are preferably arranged partially over and partially alongside the drying

tunnel 50. In the form shown, the first drying section, indicated generally by the reference numeral 52, contains a blower fan 54, and an outlet stack 56 is provided for permitting exit of a portion of the circulating gases, the exit of gases being regulated by the damper 58.

Inlet stack 60 supplies air for combustion and delivery thereof to the gas burners 62. A number of such burners are arranged across the width 10 of the drier. In the form shown five of such burners are provided, the same being regulated as to supply of combustible mixture of gas and air by the thermostatically operated controls 70 and the valves 72. As indicated by the arrows on 15 Fig. 4, the passage of circulating gases is in the first drier section 52 counter to the direction of travel of the sheet 30. The means provided for travelling sheet 30 through the tunnel drier preferably comprises the wire belt 74, which may advantageously be of the double spiral, or hinged spiral type well known for such use, the same being carried at the entrance end of the drier around the tail roll 78, and at the opposite ends of the drier carried by a corresponding head roll, not shown. The belt 74 for carrying the sheet 20 through the drier is fairly substantial and the spirals thereof made of fairly heavy wire, and such belt affords quite a considerable shielding to the under side of the sheet 30, as it passes 25 through the drier, this shielding effect being increased by the relatively closely spaced rollers 80 on which the upper run of the drier belt 74 is supported as it passes through the drier. The return run 82 of the drier belt 74 is supported 30 by the rollers 84, which however do not need to be so closely spaced. The succeeding sections of 35 the tunnel hot air drier which is preferably of the single pass variety, are preferably arranged to direct the circulating gases so that the same 40 pass through the tunnel 50 in the same direction as the sheet 30. As already stated, but one such further section is shown, and same is illustrated generally by the reference character 86.

As shown in the cross-sectional view of Fig. 5, 45 the preferred arrangement for the delivery of circulating gases to the drier tunnel 50 is such that the gases delivered from the circulating fans and heated by the gas burners are supplied to a conduit 90 which has branches 92 and 94 to the 50 opposite sides of the tunnel 50, and gases are directed into the tunnel 50 by means of nozzles 96 and 98 arranged to supply said gases above and below the sheet 30 respectively.

Except as they are combined with the provision 55 made for spraying water, preferably water containing a percentage of soluble fire arresting material, upon the sheet before it is dried, the particular construction and arrangement of the Fourdrinier apparatus and the drying apparatus 60 constitute no part of the present invention, and various other forms of apparatus suited for these purposes can be utilized.

The water delivery means are located over the sheet 30 on the Fourdrinier wire and are located 65 at such a distance from the entrance to the drier as to give opportunity for the water to even out and penetrate into the upper part of the sheet 30 before it reaches the drier. The preferred relationship is substantially as shown in Fig. 1.

The provision which is made for delivering the water, preferably containing fire resistant materials in solution, on the sheet may be of various kinds, but the preferred form shown in the drawing consists of a transverse pipe 100, which is 70 of relatively large diameter, so that its contents 75

can be held at substantially uniform pressure throughout its length, and this pipe 100 is provided with a series of spaced spray nozzles 102, 102. These nozzles 102 are arranged to secure a uniform delivery of the fluid upon the sheet when the pipe 100 is located relatively close to the sheet 30. These spray nozzles can be directed laterally and downwardly as indicated at 104, Fig. 1. A convenient mode of securing uniform distribution of fluid from each of the nozzles 102, consists in the formation thereof as simple spray nozzles centrally bored at 106, and selection thereof to give substantially identical nozzle openings adapted for uniform fluid delivery. A convenient mode of testing the fluid delivery is by supplying fluid to the nozzles at uniform pressure, which is substantially the pressure used in operation, and causing each nozzle to discharge into a graduate for a selected period of time, and selecting from the supply of nozzles those which deliver substantially equal quantities of water in such time.

While it is not essential in all cases to supply dissolved fire resistant materials with the spray water, it is preferred to incorporate a small percentage of such material with the water to be sprayed on the sheet. The preferred material for this purpose is boric acid which is not decomposed under the conditions encountered in the drier, even though the temperature in the first section of the drier, which is the most highly heated section, may be as high as 750 or 800° F. The advantages obtained by spraying water alone on the sheet and especially the avoidance of char are heightened by the use of material such as boric acid, but very good results can be obtained with the use of water alone, and water may be used with or without the addition of the chemical fire retarding agents.

The advantages obtained by the present invention consist primarily in making it possible to secure desirably higher speeds of travel of the sheet being formed and dried, and the production of a good quality, acceptable, finished sheet product at such increased production speeds.

The advantages secured will be clearly understood from the following comparison of operation with and without the water spray respectively:

Using the water spray, the apparatus is operated under speed and temperature etc. conditions adapted to produce a good, acceptable sheet which is substantially bone dry at the exit end of the drier. The sheets of distended fibrous material are very light, weighing only a few ounces per square foot. Dried with the use of the water spray, the sheet is light-colored and free from char.

If, then, for testing the effect of the water spray, the operation is continued, with no change other than that the water spray is temporarily cut off, as for example cut off during the time that a section of sheet 30, perhaps 25 feet in length, has passed through the drier, it will be found that when that part of the sheet to which added water was not supplied issues from the drier, instead of being light colored and free from charring on the upper surface as before, this part of the sheet will have a charred surface, and the interior of the sheet, instead of being substantially bone dry, will contain sufficient moisture so as to be perceptibly damp to the touch. Furthermore, the undried part of the sheet so produced, even if the sheet is subsequently further dried, is defective and unacceptable for pur-

poses for which good uniform sheets are desired. The portions of the material which have gone through the drier without being thoroughly dried are relatively much more weak and fragile than the remainder of the sheet, and cause a considerable reduction in the strength and resistivity of the whole sheet. If, for example, such partly undried sheets are stacked on one another until any considerable weight is imposed on the lower sheets in the stack, the undried parts will collapse, which, of course, ruins the sheet for commercial purposes. The sizing material used, and preferably consisting of wax or resin sizes, are less effective in such undried portions than in the parts of the sheet which have been thoroughly dried in the drier.

Without commitment to particular theory, it appears that the beneficial effects of the spraying of the water on the sheet prior to delivery thereof to the drier may be explained as follows: When the sheet is first formed on the Fourdrinier wire, it consists of an evenly distributed mixture of water, fiber and fine air bubbles. As the sheet proceeds along the Fourdrinier wire a considerable proportion of the water drains from it, passing through the wire mesh to drain pans beneath. When no spray is used, upon entering the drier the amount of water remaining in the sheet is least at and near the upper surface. This upper part of the sheet having low water content, has poor heat conduction properties. As a result of this uneven distribution of water in the sheet, the upper portion of the sheet containing least water is very difficult to dry by reason of its low heat conductivity.

When the sheet with the water so unevenly distributed, that is to say, with much less water at and near the top than at and near the lower surface, is exposed to the hot gases in the drier, the sheet will dry very rapidly on the extreme upper surface, which then becomes even less heat conductive. This further retards the passage of heat into the sheet from above to evaporate the water within the sheet, and upon continued exposure to the hot circulating gases of the drier, the top surface will scorch and char before the water is removed from the center of the sheet through application of heat from above.

While this is going on near the upper surface of the sheet, a substantially efficient drying is being performed at and near the lower surface of the sheet, which has relatively high heat conduction properties due to presence of water. With such efficient drying operation taking place at the lower part of the sheet, any tendency to scorch in this lower part is reduced by the sheet being protected by the spiral link belt of the drier and by the relatively closely spaced rollers over which the belt is passed. Another factor which tends both to efficient drying and protection from charring at the bottom of the sheet appears to consist in the further protection afforded by the presence of water vapor in substantial quantities as the drying proceeds.

The conditions just described are present and the effects just described are obtained when the sheet is passed into the drier without auxiliary spray treatment of its upper surface. Quite different conditions and results are obtained when the spray is used, and the explanation thereof appears to be as follows: The spray creates on the upper surface and in the upper portion of the sheet a condition with respect to water content generally similar to that just described as existing normally at or near the lower surface

of the sheet, or in other words, a more even distribution of water from bottom to top of the sheet. The water in the upper portion of the sheet makes it more highly heat conductive. A better and more rapid water removal from the interior of the sheet takes place from above. Also, water vapor formed over the sheet during the drying operation appears to protect the upper surface against the scorching and charring that would take place without use of the spray.

The inclusion of various fire retardant chemicals of which boric acid is an example, serves to increase the protection afforded against char. The quantity of water to be sprayed on the sheet and the amount of boric acid or equivalent fire resisting material to be included will vary considerably under varying conditions and with different thicknesses of sheet. However, it may be stated, for example, that when making a sheet eight feet wide and substantially one inch thick, and operating the apparatus at a speed of approximately eight feet per minute with a temperature of approximately 750° F., in the first drying zone, and progressively lower temperatures in subsequent zones, excellent effects can be obtained by delivery of water to the upper surface of the sheet at the rate of approximately 1.2 gallons per minute, and a desirable proportion of boric acid for use therewith is in the neighborhood of from .2% to .5% on the quantity of water sprayed, or an average of approximately .35%. It is a feature of great advantage that the use of the spray as has been described permits use of much higher drying temperatures than without the spray, and makes it possible to operate at increased speed, giving greatly increased production of good quality and commer-

cially acceptable product with use of drying apparatus which would otherwise have to be operated at lower drying temperatures and much lower speed and output.

5 We claim:

1. Process of treating relatively thick wet sheet material containing fibers held in distended relationship by relatively stable bubbles, which comprises delivering added water to the upper

10 part of the sheet, and then drying the sheet by directing hot circulating gases toward the sheet surface to obtain uniform and increased speed in drying of the sheet whereby the fibers are substantially fixed in their distended relationship and improved strength obtained with substantially no charring.

2. The process of treating relatively thick wet sheet material containing fibers held in distended relationship by relatively stable bubbles, which comprises delivering added water to the upper

20 part of the sheet substantially uniformly throughout its area, and then drying the sheet by directing hot circulating gases toward the upper and lower surfaces of the sheet to obtain uniform and increased speed in drying of the sheet whereby the fibers are substantially fixed in their distended relationship with substantially no charring.

3. The process of treating relatively thick wet sheet material as defined in claim 2 and in which the water contains water-soluble fire-retardant material.

4. The process of treating relatively thick wet sheet material as defined in claim 2 and in which the water contains boric acid in solution.

OTTO J. KRUEGER.  
JOHN CARESIO.